

## UNITED STATES PATENT OFFICE

2,303,477

## TANNING AND DYEING LEATHER

Donald Taylor Kirby, Wilmington, Del., assignor  
to E. I. du Pont de Nemours & Company, Wil-  
mington, Del., a corporation of Delaware

No Drawing. Application July 3, 1941,  
Serial No. 401,005

8 Claims. (CL 149—5)

This invention relates to a process for the tanning and dyeing of leather. Heretofore leather has been customarily tanned and dyed in separate processes. In my invention the tanning and dyeing of leather is carried out in a single process which produces a better leather and a better dyeing.

Although there are many points of particular novelty in my process, my process may be said to consist in general of partially tanning the skin in a chrome tan bath containing sodium formate, dyeing the skin with an acid dye, and completing the chrome tanning of the leather. The term "acid dye" is variously defined in the literature of the prior art, but in connection with my invention the acid dyes are described as water-soluble, non-basic dyestuffs whose individual molecules contain at least one acid group such as  $-\text{SO}_3\text{X}$ ,  $\text{OSO}_3\text{X}$ ,  $-\text{COOX}$ ,  $-\text{C}\text{—OX}$ ,  $-\text{SO}_2\text{N}(\text{X})\text{SO}_2-$ , in which formulae  $\text{X}$  is hydrogen, alkali metal, ammonia or substituted ammonia. It is believed that this definition includes the classes called "acid dyes" by the various authorities as well as certain classes not ordinarily considered acid by some authorities. The following dyestuffs are illustrative of those which are useful: Pontachrome Brown G (C. I. No. 238), Pontachrome Blue Black R Conc. (C. I. No. 202), Pontacyl Blue Black SX (C. I. No. 246), Pontacyl Brilliant Blue A (C. I. No. 714), Pontacyl Carmine 6B (C. I. No. 57), Pontacyl Dark Green B (C. I. No. 247), Pontacyl Fast Black BBO (C. I. No. 307), Pontacyl Fast Blue 5R (C. I. No. 289), Pontacyl Fast Violet 10B (C. I. No. 696), Pontacyl Green BL Conc. (C. I. No. 666), Pontacyl Navy Blue M4B (C. I. No. 304), Du Pont Orange II Conc. (C. I. No. 151), Du Pont Orange RO (C. I. No. 161), Du Pont Quinoline Yellow Conc. (C. I. No. 801), Pontamine Blue BB Supra Conc. (C. I. No. 406), Pontamine Blue RW (C. I. No. 512), Pontamine Brown D3GN (C. I. No. 596), Pontamine Diazo Black BHSW Conc. (C. I. No. 401), Pontamine Fast Red F (C. I. No. 419), Pontamine Fast Scarlet 4BS (C. I. No. 326), Pontamine Green Bx (C. I. No. 593), Pontamine Orange R (C. I. No. 415), Pontamine Sky Blue 5BX (C. I. No. 520), Pontamine Steel Blue G (C. I. No. 590), Pontamine Yellow CH (C. I. No. 365), Du Pont Resorcin Brown 5G (C. I. No. 234), Du Pont Stilbene Yellow G Conc. (C. I. No. 620), O-amino phenol→resorcin; O-amino phenol→resorcin, coppered; p-disulfanilamide  $\rightleftharpoons$  (p-cresol)<sub>2</sub>, and p-amino salicylic acid→resorcinol→picramic acid.

For practical purposes my process begins with a pickled skin. One may start with a skin at an earlier stage of its preparation but it must be brought through the various stages up to and including pickling in order to obtain optimum results so the process will be described as applied to a skin which has been pickled.

In one of the examples fleshing is carried out during my process, but it is frequently desirable to complete the fleshing prior to the commencement of the process.

The chromium salts which are used in my process are those which are customarily used in chrome tanning. Those which are listed in this specification are merely exemplary. The sodium formate, whose use is referred to in the specification, is merely exemplary of the alkali metal salts of organic acids such as sodium acetate and sodium lactate, sodium oxalate, sodium glycolate and sodium adipate, and the other alkali metal salts of these or other organic acids. In the literature these agents are called masking agents or buffering agents and their function in this process is to give added penetration and shorten the time required in the process.

As a part of my invention I have devised a new method of preparing a tan bath which has considerable advantages. It involves, generally speaking, the boiling of the chrome tanning material in a volume of water less than that which has heretofore been used, allowing the boiled tan bath to stand for some time, for instance, overnight, and extending by the addition of water. During the period of standing crystals tend to form in the concentrated liquor, which dissolve easily on extension of the bath with water.

The method of preparing the tan bath is illustrated by the following example:

40 108 pounds of commercial basic chromium sulfate are dissolved in 25 gallons of boiling water. 65 pounds of solid sodium formate (or substitute) are added. The solution is boiled five minutes. It is allowed to cool and stand overnight. Crystals are formed in this liquor. The liquor is extended to the order of 80 gallons and heated to about 80° F. before use in the tan bath. The crystals are dissolved in this operation.

The following examples illustrate the invention. The quantities are by weight and they and the details of the process are illustrative, not limitative.

*Example I*

50 Nine hundred pounds of bated domestic sheepskin which had been degreased and which had

been pickled with sulfuric acid and common salt and which had a pH value of about 2.0 as determined by spotting with a 0.04% solution of thymol blue were treated for 10 minutes in a revolving tanning drum at a temperature of 80° F. with a solution prepared by dissolving 45 pounds of common salt in 20 gallons of water.

A tanning bath was prepared by boiling together in 15 gallons of water 63 pounds of commercially prepared basic chromium sulfate (containing 23.2% of chromium calculated as Cr<sub>2</sub>O<sub>3</sub>) and 31 pounds of sodium formate and allowing to stand and cool overnight. It was extended by the addition of 40 gallons of water and was admitted, after heating, through the hollow trunnion to the revolving drum containing the sheepskins. The sheepskins were allowed to drum in the tanning bath at a temperature of 80° F. for 90 minutes, after which they had a pH value of about 3.8 as determined by spotting with an 0.04% solution of Bromphenol Blue.

An alternative method of preparing the tan bath was to boil the chromium sulfate and sodium formate in 40 gallons of water and cool to a temperature of 80° F., immediately injecting it into the tanning drum. This alternative method is not preferred.

A solution was prepared by dissolving 11 pounds of sodium bicarbonate in 10 gallons of water at 80° F., and poured through the hollow trunnion into the revolving drum containing the partially tanned sheepskins, the drumming being continued at a temperature of 80° F. for 30 minutes. After that drumming period the partially tanned sheepskins had a pH value of about 4.5 as determined by spotting with an 0.04% solution of Bromcresol Green.

The partially tanned sheepskins were removed from the tanning drum and refleshed (excess adipose tissue being removed from the flesh surfaces of the skin in the process called shaving). Fleshing is usually completed before tanning begins, but in this process it is advantageous in the securing of optimum results to be sure that the adipose tissue is completely removed. The fleshed, partially-tanned sheepskins were returned to the tanning drum, which was fitted with a perforated door, and revolved, water at 80° F. being flowed through it for 15 minutes. Excess liquor was drained from the drum, and the perforated door was replaced by a solid door.

A dye bath was prepared by boiling together in 30 gallons of water 36 pounds of a mixture of dyestuffs comprising 35 parts of Pontamine Brown RMR (C. I. No. 420), 35 parts of Pontachrome Brown RH Conc. (Mordant Acid dye, Pr. 5), 15 parts of Pontamine Brown NCR (C. I. No. 596), 10 parts of Pontamine Green S. Conc. (C. I. No. 583) and 5 parts of Pontacyl Fast Red AS Conc. (C. I. No. 176). The dyestuff solution was allowed to cool to 110° F. A solution was prepared by dissolving in 30 gallons of water at 110° F. 36 pounds of quebracho tanning extract, and the two solutions were combined and added, in one addition through the hollow trunnion, to the revolving drum containing the rinsed, fleshed, partially tanned sheepskins, which were allowed to drum therein at a temperature of 110° F. for 30 minutes.

A solution was prepared by dissolving 9 pounds of muriatic acid (approximately 32% hydrochloric acid) in 10 gallons of water at a temperature of 80° F., and added, in one addition through the hollow trunnion, to the revolving drum. The drumming was continued for 15

minutes, the solid door was replaced by a perforated door, and the drum was revolved until the excess liquor had drained off.

A tanning bath was prepared by boiling together in 6 gallons of water 27 pounds of commercially prepared basic chromium sulfate (containing 23.2% of chromium calculated as Cr<sub>2</sub>O<sub>3</sub>) and 13.5 pounds of sodium formate and allowed to stand overnight. It was extended with 40 gallons of water, and added, in one addition through the hollow trunnion, to the resealed revolving drum containing the dyed partially-tanned sheepskins. The drumming was continued at a temperature of 80° F. for 60 minutes.

A solution was prepared by dissolving in 10 gallons of water at a temperature of 80° F. 5 pounds of sodium bicarbonate, and added, in one addition through the hollow trunnion, to the revolving drum containing the dyed, completely-tanned sheepskins. The drumming was continued for 30 minutes at a temperature of 80° F., the solid door of the drum was replaced by a perforated door, water at a temperature of 100° F. was allowed to flow through the revolving drum for 30 minutes, the temperature of the rinsing water was raised to 140° F. and the rinse was continued for 10 minutes.

An emulsion was prepared by stirring into 60 gallons of water at 140° F. 20 pounds of commercially prepared fatliquor (comprising approximately 65% sulfonated cod oil, 15% unsulfonated cod oil and 20% water), and added, in one addition through the hollow trunnion, to the resealed revolving drum containing the rinsed, dyed, completely-tanned sheepskins. The drumming was continued for 30 minutes. The sheepskins were removed from the drum and hosed-up to drain.

The fatliquored, dyed, completely-tanned sheepskins were finished by methods known to be appropriate to the finishing of chrome tanned leather.

The leather prepared by this process may be used as chrome-tanned grain sheepskin garment leather. The usual methods employed in the preparation of this type of leather involve either fully chrome tanning, dyeing, fatliquoring, drying and finishing, or chrome tanning, further tanning with vegetable extracts or synthetic tanning agents of the type represented by sulfonated phenol-formaldehyde condensation products, fatliquoring, drying, rewetting, dyeing, drying and finishing. The second of these known processes yields leather and shade characteristics better than that produced by the other and is usually employed for the preparation of the better grade of garment leathers. The method described in Example I hereof produces leather having characteristics superior to those that can be obtained by either of the known general methods and produces it more economically. This leather is characterized by having a higher tensile strength, a full, "round," soft and uniform feel, and a full, level and fast brown color. The higher tensile strength is evidenced in the markedly decreased number of "tear offs" in the subsequent staking operation. This reduction of "tear offs" represents an economy by the reduction of damage to the leather in processing. A fuller shade is obtained by this method than by the methods that involve fatliquoring, drying, and rewetting before dyeing. A more level shade of color is obtained by my method. A more uniform color is obtained among the various skins of a group than among a similar group prepared by the known methods. There is a marked re-

duction of darker colored imperfections on the grain of the skins. The color is faster to washing.

The percentage of first grade grain sheepskin garment leather usually prepared from low grade domestic sheepskins by the known methods is normally approximately 5%. The percentage of first grade leather produced by this example is increased to approximately 15%. The percentage of low grade leather is reduced markedly. The improved leather characteristics represent a marked increase in value.

A decided economy in time, equipment and expense is effected by this invention since a dyed leather having superior properties can be prepared in less than one-half the normal time required for the known process involving dyeing after crusting (drying). My process is faster than either of the prior processes briefly described above.

A known method of preparing leather included basic chromium salts and an organic acid salt in the tan bath, and dyed after tanning, or after crusting and rewetting.

The shade of the dyed leather obtained by the method of the example has superior levelness, fastness, and uniformity compared to the shade obtained by the said prior process. The uniformity from skin to skin, the roundness, softness, and uniformity of the leather are also improved.

This process is not to be confused with the older and inferior process of tanning completely, dyeing, and retaining.

The physical characteristics of the leather prepared by this and other examples may be altered by varying the amount and kind of organic acid alkali metal salt used in either of the tanning baths. For example, if 50 pounds of sodium formate are used in the first bath, the resulting leather will be plumper and softer than that resulting from the use of 31 pounds of sodium formate. If 25 pounds of sodium formate are used, the resulting leather will be thinner and boardier than if 31 pounds are used. Corresponding alterations in the physical characteristics of the leather may be obtained by varying the amount of masking agent used in the second tanning bath. The sodium formate used in either or both tanning baths may be replaced by varying amounts of other alkali metal salts of organic acids, such as sodium acetate, or lactate or oxalate, etc., or mixtures of them, with consequent variation in leather properties.

Alterations in the physical characteristics of the leather may also be obtained by varying the amount of whatever chromium salt is used in the tanning baths. Increased amounts of chromium salt will produce softer, fuller leather.

In Example I 4% (on the shaved weight of the pickled sheepskin) of quebracho tanning extract is included in the dyebath. The inclusion of quebracho tanning extract helps to impart a full, soft, "round" feel to the leather. The amount of quebracho tanning extract may be raised as high as 12% (on the shaved weight of pickled sheepskin), or it may be omitted from the dyebath. Varying degrees of softness, fullness and "roundness" of feel may be obtained by varying the amount of quebracho tanning extract. Instead of quebracho tanning extract, natural tanning extracts may be included in the dyebath with a change in result. For instance, if hemlock tanning extract is substituted for quebracho tanning extract (on a part-for-part

basis), firmer, less plump, less "round" feeling leather will be obtained. Amounts of extract from 0-12% on the shaved weight of pickled sheepskin produce useful results. Examples of useful extracts are quebracho, hemlock, sumac, gambier, logwood, divi-divi, oak bark, mangrove, wattle bark, spruce bark, and valonia. They are used alone or in combination. The inclusion of vegetable tanning extracts in the dyebath is not necessary for the operation of the examples, but their inclusion frequently produces useful characteristics in the leather. Synthetic tanning agents may be included in the dyebath in addition to, or instead of, vegetable tanning extract.

For instance, from 0-5% of the following of synthetic tanning agents may be included: sulfite cellulose waste liquor, sulfonated phenol-formaldehyde condensates or sulfonated cresol formaldehyde condensates.

The dyebath used in Example I contained 4% (on the shaved weight of pickled sheepskin) of a mixture of synthetic dyestuffs. The amount of dyestuff may be altered to obtain various depths of color.

The dyestuffs, when applied according to the foregoing directions, affix themselves principally to the grain and flesh surfaces of the skins, there being only slight penetration of the color to the interior of the skins, but the extent of penetration of color may be controlled by adjusting the pH value of the partially-tanned sheepskins prior to application of the dyestuffs. If, in Example I, the pH is adjusted to pH 5.5 before application of the dyestuffs, partial penetration

of color into the interior of the skins will be obtained. If the pH value is adjusted to pH 7.0 before application of the dyestuffs, full penetration of color into the interior of the skins will be obtained. The alkali used to adjust the pH

value of the partially-tanned sheepskins need not be limited to sodium bicarbonate. Other alkalis, for example sodium hydroxide, sodium carbonate, sodium borate, ammonium hydroxide, disodium phosphate and trisodium phosphate, may be used.

The use of disodium phosphate and trisodium phosphate to adjust the pH value is not preferred, because the phosphate ion is considered to have a harmful secondary effect on the leather. If the pH value of the partially-tanned sheep-

skins is adjusted to a value higher than pH 4.5, a correspondingly larger amount of muriatic acid should be used to exhaust the dyebath. Consequently, the amount of alkali used to "set" the tannage after application of the second tanning bath should be increased. The acid used to exhaust the dyebath need not be limited to muriatic acid. Other inorganic and organic acids may be used. For example, sulfuric acid, formic acid and acetic acid.

The fatliquor used to treat the completely-tanned leather need not be limited to one having the composition mentioned in Example I. Other fatliquors suitable for treating chrome-tanned grain garment leather prepared by known methods may be used.

#### Example II

Nine hundred pounds of domestic sheepskins which have been treated in the beam house for the manufacture of glove leather and which have been pickled with sulfuric acid and common salt and which have a pH value of about 2.0 as determined by spotting with an 0.04% solution of Thymol Blue, are treated in a revolving tanning drum for 10 minutes with a solution prepared

by dissolving 45 pounds of common salt in 20 gallons of water.

A tanning bath is prepared by boiling together in 14 gallons of water 60 pounds of commercially prepared basic chromium sulfate (containing 23.2% of chromium calculated as  $\text{Cr}_2\text{O}_3$ ) and 32 pounds of sodium glycolate and allowing the resulting solution to stand overnight. It is extended with 50 gallons of water, heated at 80° F. and poured through the hollow trunnion into the revolving drum containing the sheepskins. The sheepskins are allowed to drum in the tanning bath at a temperature of 80° F. for 90 minutes. The solid door of the drum is replaced by a perforated door. The drum is revolved. Water at a temperature of 100° F. is allowed to flow through the revolving drum for 30 minutes. The partially tanned sheepskins are removed from the drum and hosed up to drain.

A dye solution is prepared by boiling 8 pounds of Pontamine Black E Double (C. I. No. 581) in 60 gallons of water and allowing the resulting solution to cool to 100° F. The drained, partially tanned sheepskins are spread on a dyeing table with their grain surfaces uppermost. The dye solution is brushed onto the grain surfaces, and the dyestuff is set by brushing the dyed surfaces with a 1% solution of hydrochloric acid. The dyed surfaces of the sheepskins are rinsed with water at a temperature of 100° F. The dyed, partially tanned sheepskins are returned to the tanning drum.

A tanning bath is prepared by boiling together in 7 gallons of water 30 pounds of commercially prepared basic chromium sulfate (containing 23.2% of chromium calculated as  $\text{Cr}_2\text{O}_3$ ) and 16 pounds of sodium glycolate and allowing the resulting solution to cool. The bath thus prepared is extended after the formation of crystals with 50 gallons of water and added through the hollow trunnion, to the revolving drum containing the dyed, partially tanned sheepskins. The sheepskins are allowed to drum in the tanning bath at a temperature of 80° F. for 60 minutes.

A solution is prepared by dissolving 8 pounds of sodium bicarbonate in 10 gallons of water at a temperature of 80° F. This solution is added, in one addition through the hollow trunnion, to the revolving drum containing the dyed, fully tanned sheepskins. The drumming is continued for 30 minutes at a temperature of 80° F. The solid door of the drum is replaced by a perforated door. The drum is revolved. Water at a temperature of 100° F. is allowed to flow through the revolving drum for 20 minutes. The temperature of the rinsing water is raised to 130° F. and the rinse is continued for 10 minutes. The perforated door is replaced by a solid door.

An emulsion is prepared by stirring into 60 gallons of water at a temperature of 140° F. 63 pounds of a commercially prepared fatliquor (comprising approximately 40% sulfonated cod oil, 30% unsulfonated neat's foot oil and 30% water). This emulsion is added, in one addition through the hollow trunnion, to the revolving drum containing the dyed, fully-tanned sheepskins. The drumming is continued for 30 minutes at a temperature of 130° F.

The fatliquored, dyed, fully tanned sheepskins are removed from the drum and hosed-up to drain.

The leather prepared by this process may be used in the preparation of white-backed glove leather. It is characterized by having a fuller, leveler black shade which is faster to washing

and a superior round, soft, uniform feel as compared to glove leather prepared by the known methods.

### Example III

5 Nine hundred pounds of bated domestic sheepskins which have been degreased and which have been pickled with sulfuric acid and common salt and which have a pH value of about 2.0 are treated in a revolving tanning drum for 10 minutes at a temperature of 80° F., with a solution prepared by dissolving 45 pounds of common salt in 20 gallons of water.

A tanning bath is prepared by boiling together in 15 gallons of water 63 pounds of commercially prepared basic chromium sulfate (containing 23.2% of chromium calculated as  $\text{Cr}_2\text{O}_3$ ) and 27 pounds of sodium oxalate and allowing the resulting solution to cool overnight. The bath thus prepared is extended with 40 gallons of water and added, in one addition through the hollow trunnion, to the revolving drum containing the sheepskins. The sheepskins are allowed to drum in the tanning bath at a temperature of 80° F. for 90 minutes. After this drumming period the sheepskins have a pH value of about 3.5 as determined with Bromphenol Blue.

A solution is prepared by dissolving 15 pounds of sodium bicarbonate in 10 gallons of water at 80° F. This solution is added, in one addition through the hollow trunnion, to the revolving drum containing the partially tanned sheepskins, and the drumming is continued for 30 minutes at a temperature of 80° F. After this drumming period the skins have a pH value of about 5.0 as determined with Bromcresol Green.

The solid door of the drum is replaced by a perforated door. The drum is allowed to revolve. Water at a temperature of 80° F. is allowed to flow through the revolving drum containing the partially tanned sheepskins for 15 minutes. Excess liquor is drained from the drum and the perforated door is replaced by a solid door.

A solution is prepared by dissolving 45 pounds of hemlock tanning extract in 30 gallons of water at a temperature of 100° F. and mixing with a solution prepared by dissolving 30 pounds of Pontamine Brown RMR (C. I. No. 420) in 30 gallons of boiling water. This combined solution is cooled to a temperature of 100° F. and added in one addition through the hollow trunnion, to the revolving drum containing the partially tanned sheepskins. The drumming is continued at a temperature of 100° F. for 30 minutes. A solution prepared by adding 9 pounds of muriatic acid (approximately 32% hydrochloric acid) to 10 gallons of water at a temperature of 80° F. is added to the drum. The drumming is continued for 15 minutes. The solid door of the drum is replaced by a perforated door. The drum is revolved. Water at a temperature of 100° F. is allowed to flow through the revolving drum for 30 minutes. The perforated door is replaced by a solid door.

A solution is prepared by dissolving 9 pounds of du Pont Basic Brown BR (C. I. No. 332) and 4 pounds of formic acid (87%) in 60 gallons of water at 100° F. This solution constitutes the dyebath. The dyebath is added, in one addition through the hollow trunnion, to the revolving drum containing the partially-tanned sheepskins. The drumming is continued at a temperature of 100° F. for 30 minutes. The solid door is replaced by a perforated door, and the drum is allowed to revolve. Water at a temperature of 100° F. is allowed to flow through the revolving

drum for 30 minutes. The perforated door is replaced by a solid door.

A solution is prepared by dissolving 45 pounds of hemlock tanning extract in 30 gallons of water at a temperature of 100° F. and mixing with a solution prepared by dissolving 30 pounds of Pontamine Brown RMR (C. I. No. 420) in 30 gallons of boiling water. This combined solution is cooled to a temperature of 100° F. and added in one addition through the hollow trunnion, to the revolving drum containing the partially tanned sheepskins. The drumming is continued at a temperature of 100° F. for 30 minutes. A solution prepared by adding 9 pounds of muriatic acid (approximately 32% hydrochloric acid) to 10 gallons of water at a temperature of 80° F. is added to the drum. The drumming is continued for 15 minutes. The solid door of the drum is replaced by a perforated door. The drum is revolved. Water at a temperature of 100° F. is allowed to flow through the revolving drum for 30 minutes. The perforated door is replaced by a solid door.

A solution is prepared by dissolving 9 pounds of Du Pont Basic Brown BR (C. I. No. 332) and 4 pounds of formic acid (87%) in 60 gallons of water at 100° F. This solution constitutes the dyebath. The dyebath is added, in one addition through the hollow trunnion, to the revolving drum containing the partially-tanned sheepskins. The drumming is continued at a temperature of 100° F. for 30 minutes. The solid door is replaced by a perforated door, and the drum is allowed to revolve. Water at a temperature of 100° F. is allowed to flow through the revolving drum for 30 minutes. The perforated door is replaced by a solid door.

A tanning bath is prepared by boiling together in 6 gallons of water 27 pounds of commercially prepared basic chromium sulfate (containing 23.2% of chromium calculated as Cr<sub>2</sub>O<sub>3</sub>) and 13 pounds of sodium oxalate and allowing the resulting solution to stand. After crystal formation and extension with 40 gallons of water the bath is poured into the revolving drum containing the partially tanned, dyed sheepskins. The drumming is continued at a temperature of 80° F. for 60 minutes.

A solution is prepared by dissolving 5 pounds of sodium bicarbonate in 10 gallons of water at 80° F. This solution is added, in one addition through the hollow trunnion, to the revolving drum containing the dyed, completely tanned sheepskins. The drumming is continued at a temperature of 80° F. for 30 minutes. The solid door of the drum is replaced by a perforated door, and water at a temperature of 100° F. is allowed to flow through the revolving drum for 30 minutes. The temperature of the rinsing water is raised to 120° F., and the rinse is continued for 10 minutes.

An emulsion is prepared by stirring into 60 gallons of water at a temperature of 120° F. 30 pounds of a partially sulfonated cod oil (comprising approximately 65% sulfonated cod oil, 15% unsulfonated cod oil and 20% water). This emulsion constitutes the flatliquor. The flatliquor is added, in one addition through the hollow trunnion, to the revolving drum containing the dyed, fully-tanned sheepskins. The drumming is continued at a temperature of 120° F. for 30 minutes. The fatliquored, dyed, tanned sheepskins are removed from the drum and hosed-up to drain.

Leather prepared by this process may be used

in preparing chrome tanned grain sheepskin garment leather. It is characterized by having a leveler and fuller brown shade which is faster to washing and a plumper, fuller, "rounder" feel than garment leather prepared by the known methods of completely tanning and dyeing; or tanning fatliquoring, crusting, rewetting and dyeing.

#### Example IV

10 Five hundred pounds of South American sheepskins which have been treated in the beam-house for the manufacture of glove leather and which have been pickled with sulfuric acid and common salt and which have a pH value of about 2.2 as determined by spotting with an 0.04% solution of Thymol Blue are treated for 10 minutes in a revolving tanning drum with a solution prepared by dissolving 25 pounds of common salt in 12 gallons of water at a temperature of 80° F.

15 A tanning bath is prepared by boiling together in 9 gallons of water 40 pounds of commercially prepared basic chromium sulfate (containing 23.2% of chromium calculated as Cr<sub>2</sub>O<sub>3</sub>) and 13 pounds of sodium adipate and allowing the solution to stand overnight. The tanning bath thus prepared is extended with 25 gallons of water and added, in one addition through the hollow trunnion, to the revolving drum containing the sheepskins. The drumming is continued at a

20 temperature of 80° F. for 90 minutes.

25 A solution is prepared by dissolving 4 pounds of sodium carbonate in 5 gallons of water at a temperature of 80° F. This solution is added, in one addition through the hollow trunnion, to the revolving drum containing the partially-tanned sheepskins. The drumming is continued, at a temperature of 80° F. for 30 minutes. The solid door of the drum is replaced by a perforated door. The drum is allowed to revolve. Water at a temperature of 100° F. is allowed to flow through the revolving drum for 30 minutes. The temperature of the rinsing water is raised to 120° F. and the rinse is continued for 30 minutes. Excess liquor is allowed to drain from the drum, and the perforated door is replaced by a solid door.

30 A solution is prepared by boiling in 35 gallons of water 15 pounds of the synthetic dyestuff—"Pontachrome" Brown G (C. I. No. 238). The solution is allowed to cool to a temperature of 120° F. and is then added, in one addition through the hollow trunnion, to the revolving drum containing the partially tanned sheepskins. The drumming is continued at a temperature of 120° F. for 30 minutes.

35 A solution is prepared by adding 5 pounds of formic acid (approximately 87%) to 5 gallons of water at a temperature of 120° F. This solution is added, in one addition through the hollow trunnion, to the revolving drum containing the dyed, partially-tanned sheepskins. The drumming is continued for 20 minutes. The solid door of the drum is replaced by a perforated door, and the drum is revolved until the excess liquor has drained from the skins.

40 A tanning bath is prepared by boiling together in 4.5 gallons of water 20 pounds of commercially prepared basic chromium sulfate (containing 23.2% of chromium calculated as Cr<sub>2</sub>O<sub>3</sub>) and 6.5 pounds of sodium adipate and allowing the solution to cool to a temperature of 80° F. This tanning bath is added, after extension with 25 gallons of water, to the revolving drum containing the dyed, partially-tanned sheepskins. The

drumming is continued at a temperature of 80° F. for 60 minutes.

A solution is prepared by dissolving 6 pounds of sodium carbonate in 5 gallons of water at a temperature of 80° F. This solution is added, in one addition through the hollow trunnion, to the revolving drum containing the dyed, fully-tanned sheepskins. The drumming is continued for 30 minutes. The solid door of the drum is replaced by a perforated door, and the drum is allowed to revolve. Water at a temperature of 100° F. is allowed to flow through the revolving drum for 30 minutes. The temperature of the rinsing water is raised to 140° F. and the rinse is continued for 10 minutes. The perforated door of the drum is replaced by a solid door.

An emulsion is prepared by stirring into 35 gallons of water at 140° F. 18 pounds of commercially prepared fatliquor (comprising approximately 65% sulfonated cod oil, 15% unsulfonated cod oil and 20% water). This emulsion is added, in one addition through the hollow trunnion, to the revolving drum containing the dyed, fully-tanned sheepskins. The drumming is continued for 30 minutes. The fatliquored, dyed, fully-tanned sheepskins are removed from the drum and hosed-up to drain.

The leather prepared by this example may be used as chrome-tanned grain glove leather. It is characterized by having a fuller, rounder, softer, silkier feel, a leveler tan color which is faster to washing and a grain surface with less evidence of imperfections than glove leather prepared by the known methods of manufacture.

#### Example V

Nine hundred pounds of Persian goatskins which have been processed in the beam house for the manufacture of sueded leather and which have been pickled with sulfuric acid and common salt and which have a pH value of about 2.2 are treated in a revolving tanning drum at a temperature of 80° F. for 10 minutes with a solution prepared by dissolving 45 pounds of common salt in 20 gallons of water.

A tanning bath is prepared by boiling together in 12.5 gallons of water 54 pounds of commercially prepared basic chromium sulfate (containing 23.2% of chromium calculated as Cr<sub>2</sub>O<sub>3</sub>) and 30 pounds of sodium acetate and allowing the solution to stand overnight. After extension with 40 gallons of water, this bath is added to the revolving drum containing the goatskins. The drumming is continued for 90 minutes at a temperature of 80° F.

A solution is prepared by dissolving in 10 gallons of water at a temperature of 80° F. 10 pounds of sodium bicarbonate. This solution is added, in one addition through the hollow trunnion, to the revolving drum containing the partially-tanned goatskins. The drumming is continued for 30 minutes at a temperature of 80° F. The solid door of the drum is replaced by a perforated door. The drum is revolved. Water at a temperature of 100° F. is allowed to flow through the revolving drum for 30 minutes.

The partially-tanned goatskins are removed from the drum, "wet-wheeled" (buffed) and returned to the drum.

A solution is prepared by boiling in 30 gallons of water 63 pounds of the synthetic dyestuff: Pontamine Brown RMR Conc. (C. I. No. 420). The dyestuff solution is allowed to cool to a temperature of 120° F. A solution is prepared by dissolving in 30 gallons of water 25 pounds of

hemlock tanning extract and 20 pounds of sumac tanning extract. The dyestuff solution and tanning extract solution are combined and added, in one addition through the hollow trunnion, to the revolving drum containing the partially-tanned goatskins. The drumming is continued at a temperature of 120° F. for 30 minutes.

A solution is prepared by adding to 10 gallons of water at a temperature of 120° F. 10 pounds of muriatic acid (approximately 32% hydrochloric acid). This solution is slowly added through the hollow trunnion to the revolving drum containing the dyed, partially-tanned goatskins. The drumming is continued at a temperature of 120° F. for 30 minutes. The solid door of the drum is replaced by a perforated door. The drum is revolved until the excess liquor has drained from the skins. The perforated door is replaced by a solid door.

A tanning bath is prepared by boiling together in 4 gallons of water 18 pounds of commercially prepared basic chromium sulfate (containing 23.2% of chromium calculated as Cr<sub>2</sub>O<sub>3</sub>) and 9 pounds of sodium acetate and allowing the solution to stand until crystals form. 40 gallons of water are added, and the solution is poured into the revolving drum containing the dyed, partially-tanned goatskins. The drumming is continued at a temperature of 80° F. for 60 minutes.

A solution is prepared by dissolving in 10 gallons of water at a temperature of 80° F. 7 pounds of sodium bicarbonate. This solution is added, in one addition through the hollow trunnion, to the revolving drum containing the dyed, completely-tanned goatskins. The drumming is continued at a temperature of 80° F. for 30 minutes. The solid door of the drum is replaced by a perforated door. The drum is revolved. Water at a temperature of 100° F. is allowed to flow through the drum for 20 minutes. The temperature of the rinsing water is raised to 140° F. and the rinse is continued for 10 minutes. Excess liquor is drained from the drum, and the perforated door is replaced by a solid door.

An emulsion is prepared by stirring into 50 gallons of water at a temperature of 140° F. 45 pounds of commercially prepared fatliquor (comprising approximately 30% sulfonated cod oil, 20% unsulfonated neat's foot oil and 50% water). This emulsion is added in one addition through the hollow trunnion, to the revolving drum containing the dyed, completely-tanned goatskins. The drumming is continued for 30 minutes.

The fatliquored, dyed, completely-tanned goatskins are removed from the drum and hosed-up to drain. The drained leather is dried in a drying-tunnel. After it has become thoroughly dry, the leather is moistened in damp sawdust and buffed.

Leather prepared by this process may be used in preparing sueded chrome-tanned goatskin leather. It is characterized by a level brown color and a plump, full, "round" feel. Sueded goatskin leather prepared by orthodox chrome-tanning methods is "pearled" (a term describing treatment with materials such as flour and egg yolk), crusted, (dried) and wet-back before it is dyed. These operations consume several days. By the method of this example these time-consuming operations are eliminated. The shade is leveler than normally obtained by the orthodox method.

#### Example VI

Two hundred pounds of drained, shaved Persian kidskins which have been pickled with sulfuric

acid and common salt and which have a pH value of about 2.0 are treated for 10 minutes at a temperature of 80° F. in a revolving tanning drum with a solution prepared by dissolving 10 lbs. of common salt in 4 gallons of water.

A tanning bath is prepared by boiling together in 3.75 gallons of water 16 pounds of commercially prepared basic chromium sulfate (containing 23.2% chromium calculated as Cr<sub>2</sub>O<sub>3</sub>) and 9.5 pounds of sodium formate and allowing the resulting solution to stand. The bath thus prepared is extended with 22 gallons of water and added, in one addition through the hollow trunnion, to the revolving drum containing the kidskins. The kidskins are allowed to drum in the tanning bath at a temperature of 80° F. for 90 minutes. At the end of this drumming period the kidskins have a pH value of about 4.2.

A solution is prepared by dissolving 20 ounces of sodium bicarbonate in one gallon of water at a temperature of 80° F. This solution is added, in one addition through the hollow trunnion, to the revolving drum containing the partially-tanned kidskins. The partially-tanned kidskins are allowed to drum in the sodium bicarbonate solution at a temperature of 80° F. for 15 minutes. A solution is made by dissolving 20 ounces of sodium bicarbonate in one gallon of water at a temperature of 80° F. This solution is added, in one addition through the hollow trunnion, to the revolving drum containing the partially-tanned kidskins. The partially-tanned kidskins are allowed to drum in the sodium bicarbonate solution for 25 minutes at a temperature of 80° F.

The solid door of the drum is loosened and the excess liquor is allowed to drain from the drum. The solid door of the drum is replaced by a perforated door. Fifty gallons of water at 80° F. are added to the drum through the hollow trunnion. The drum is revolved for five minutes to allow the excess liquor to drain from the partially-tanned kidskins.

A solution is made by dissolving 20 fluid ounces of commercial ammonium hydroxide (approximately 35%) in 4 gallons of water at 100° F. This solution is added, in one addition through the hollow trunnion, to the revolving drum containing the partially-tanned kidskins. The partially-tanned kidskins are drummed in the ammonia solution for three minutes at a temperature of 100° F.

A solution is prepared by boiling together in 20 gallons of water the following synthetic dyestuffs — 4 pounds 12 ounces of du Pont Resorcin Brown 5G (C. I. No. 234), 2.5 ounces of Pontamine Green S Conc. (C. I. No. 583), 6.5 ounces of Pontamine Green BX (C. I. No. 593), 5.2 ounces of Pontamine Brown NCR (C. I. 596), 13 ounces of Pontamine Brown RMR (C. I. No. 420), 13 ounces of Pontachrome Brown RH Conc. (a mordant acid dye) and one ounce of Pontacyl Fast Red AS Conc. (C. I. No. 176). The solution is allowed to cool to a temperature of 100° F. Eight pounds of quebracho tanning extract and eight pounds of gambier tanning extract are mixed together and added to the solution of synthetic dyestuffs at 100° F. The resulting solution constitutes the dyebath. The dyebath is added, in one addition through the hollow trunnion, to the revolving drum containing the partially-tanned kidskins. The partially-tanned kidskins are drummed in the dyebath for 40 minutes at a temperature of 100° F.

A solution is prepared by dissolving 32 fluid

ounces of muriatic acid (approximately 32% HCl) in four gallons of water at a temperature of 80° F. This solution is slowly added through the hollow trunnion to the revolving drum containing the dyed, partially-tanned kidskins. The drumming is continued for 15 minutes at a temperature of 80° F.

The solid door of the drum is replaced by a perforated door and the drum is revolved for three minutes. The perforated door is replaced by a solid door.

A tanning bath is prepared by boiling together in 2 gallons of water 8 pounds of commercially prepared basic chromium sulfate (containing 23.2% of chromium calculated as Cr<sub>2</sub>O<sub>3</sub>) and 4 pounds 13 ounces of sodium formate and allowing the resulting solution to stand. This tanning is extended with 18 gallons of water and added, in one addition through the hollow trunnion, to the revolving drum containing the dyed, partially-tanned kidskins. The drumming is continued for 60 minutes at a temperature of 80° F.

A solution is prepared by dissolving 14.5 ounces (avoird.) of sodium bicarbonate (NaHCO<sub>3</sub>) in 2 gallons of water at 80° F. This solution is added, in one addition through the hollow trunnion, to the revolving drum containing the dyed, fully-tanned kidskins. The drumming is continued for 15 minutes at a temperature of 80° F. A solution is prepared by dissolving 14.5 ounces (avoird.) of sodium bicarbonate in 2 gallons of water at 80° F. This solution is added, in one addition through the hollow trunnion, to the revolving drum containing the dyed, fully-tanned kidskins. The drumming is continued for 25 minutes. The door of the drum is removed and the excess liquor is allowed to drain from the skins.

The drum is fitted with a perforated door. Water at 80° F. is allowed to flow through the revolving drum containing the dyed, partially-tanned kidskins for 20 minutes. The temperature of the rinsing water is raised to 130° F., and the rinse is continued for 20 minutes. The perforated door is replaced by a solid door.

An emulsion is prepared by stirring 3 pounds of commercially prepared sulfonated cod oil into 18 gallons of water at 130° F. This emulsion constitutes the fatliquor. The fatliquor is added, in one addition through the hollow trunnion, to the revolving drum containing the rinsed, dyed, fully-tanned kidskins. The drumming is continued for 30 minutes at a temperature of 130° F. The kidskins are removed from the drum and hoisted-up to drain.

The fully-tanned, dyed, fatliquored kidskins are dried, dampened, dry-milled, staked, tacked-out and finished by known methods.

The kidskins treated by this process may be used for chrome-tanned grain kidskin shoe upper leather. The leather prepared according to this process is characterized by a fuller, softer, rounder feel and a fuller, leveler brown color which is faster to washing than dyed leather prepared by the known methods of completely tanning and subsequently dyeing.

#### Example VII.

Twenty-five pounds of peccary skins which have been treated in the beam house for the manufacture of glove leather and which have been degreased and which have been pickled with sulfuric acid and common salt are treated in a revolving tanning drum for 10 minutes with

a solution prepared by dissolving 2.5 pounds of common salt in one gallon of water at a temperature of 80° F.

A tanning bath is prepared by boiling together in .75 gallon of water 2.5 pounds of commercially prepared basic chromium sulfate (containing 23.2% of chromium calculated as  $\text{Cr}_2\text{O}_3$ ), 10 ounces of sodium acetate and 10 ounces of sodium lactate and allowing the solution to cool. After extension with 3 gallons of water, the tanning bath is added, in one addition through the hollow trunnion, to the revolving drum containing the peccary skins. The drumming is continued for 90 minutes at a temperature of 80° F.

A solution is prepared by dissolving 6 ounces (avoird.) of sodium bicarbonate in one-half gallon of water at a temperature of 80° F. for 30 minutes.

The solid door of the drum is replaced by a perforated door. The drum is revolved. Water at a temperature of 100° F. is allowed to flow through the revolving drum containing the partially-tanned peccary skins for 20 minutes. The temperature of the rinsing water is raised to 120° F. and the rinse is continued for 10 minutes. The excess liquor is drained from the drum, and the perforated door is replaced by a solid door.

A solution is prepared by boiling together in 3 gallons of water 12 ounces of sodium bicarbonate, 6 ounces of Pontachrome Brown G (C. I. No. 238) and 2 ounces of Pontachrome Brown RH Conc. (a mordant acid dyestuff). This solution constitutes the dyebath. The dyebath at a temperature of 110° F. is added, in one addition through the hollow trunnion, to the revolving drum, containing the partially-tanned peccary skins. The drumming is continued at a temperature of 110° F. for 30 minutes.

A solution is prepared by dissolving 12 ounces of muriatic acid (approximately 32% HCl) in one-half gallon of water at 80° F. This solution is added, in one addition through the hollow trunnion, to the revolving drum containing the dyed, partially tanned peccary skins. The drumming is continued for 20 minutes at a temperature of 80° F. The solid door of the drum is replaced by a perforated door and the excess liquor is allowed to drain from the drum. The perforated door is replaced by a solid door.

A tanning bath is prepared by boiling together in .5 gallon of water 1.5 pounds of commercially prepared basic chromium sulfate (containing 23.2% chromium calculated as  $\text{Cr}_2\text{O}_3$ ), 7 ounces of sodium acetate and 7 ounces of sodium lactate and allowing the solution to stand several hours. The tanning bath with 2.5 gallons of water added, is poured through the hollow trunnion into the revolving drum containing the dyed, partially-tanned peccary skins. The drumming is continued for 60 minutes at a temperature of 100° F.

A solution is prepared by dissolving 5 ounces of sodium bicarbonate in one-half gallon of water at a temperature of 80° F. This solution is added, in one addition through the hollow trunnion, to the revolving drum containing the dyed, fully-tanned peccary skins. The drumming is continued for 30 minutes at a temperature of 80° F. The solid door of the drum is replaced by a perforated door. Water at a temperature of 110° F. is allowed to flow through the revolving drum containing the dyed, fully-tanned peccary skins for 20 minutes. The temperature of the rinsing water is raised to 140°

F., and the rinse is continued for 10 minutes. Excess liquor is allowed to drain from the drum. The perforated door of the drum is replaced by a solid door.

An emulsion is prepared by stirring into 2 gallons of water at 140° F. 3 pounds of commercially prepared fatliquor (comprising approximately 40% sulfonated cod oil, 30% unsulfonated neat's foot oil and 30% water. This emulsion is added, in one addition through the hollow trunnion, to the revolving drum containing the dyed, fully-tanned peccary skins. The drumming is continued for 30 minutes at a temperature of 140° F.

The fatliquored, dyed, fully-tanned peccary skins are removed from the drum and horsed-up to drain.

Leather prepared by this process may be used for chrome-tanned grain pigskin glove leather. The time required for preparing dyed leather by this process is less than one-half that required by the known process of completely tanning and subsequently dyeing. The dyed leather has a fuller, leveler, more uniform shade, and is faster to washing, plumper, softer, and of more uniform feel than leather prepared by any known method.

#### Example VIII

Nine hundred pounds of drained South American sheepskin skivers which have been treated in the beamhouse for the manufacture of glove leather and which have been pickled with sulfuric acid and common salt are treated for 10 minutes at a temperature of 80° F. in a revolving tanning drum with a solution prepared by dissolving 45 pounds of common salt in 20 gallons of water.

A tanning bath is prepared by boiling together in 17 gallons of water 72 pounds of commercially prepared basic chromium sulfate (containing 23.2% of chromium calculated as  $\text{Cr}_2\text{O}_3$ ) and 36 pounds of sodium formate and allowing the resulting solution to stand overnight. The bath thus prepared with the extension of 22 gallons of water is added in one addition through the hollow trunnion, to the revolving tanning drum containing the sheepskin skivers. The sheepskin skivers are allowed to drum in the tanning bath at a temperature of 80° F. for 90 minutes.

A solution is prepared by dissolving 11 pounds of sodium bicarbonate ( $\text{NaHCO}_3$ ) in 10 gallons of water at 80° F. This solution is added, in one addition through the hollow trunnion, to the revolving drum containing the partially-tanned sheepskin skivers. The partially-tanned sheepskin skivers are allowed to drum in the sodium bicarbonate solution at a temperature of 80° F. for 30 minutes.

The solid door of the tanning drum is replaced by a perforated door. The drum is allowed to revolve. Water at a temperature of 80° F. is allowed to flow through the revolving drum containing the partially-tanned sheepskin skivers for 20 minutes. Excess water is drained from the drum and the perforated door is replaced by a solid door.

A solution is prepared by dissolving 8 pounds of sodium bicarbonate in 10 gallons of water at 80° F. This solution is added, in one addition through the hollow trunnion, to the revolving drum containing the partially-tanned sheepskin skivers. The drumming is continued for 20 minutes at a temperature of 80° F.

The solid door of the tanning drum is replaced by a perforated door. The drum is allowed to revolve. Water at a temperature of 80° F. is al-

lowed to flow through the revolving drum containing the partially tanned sheepskin skivers for 10 minutes. Excess water is allowed to drain from the drum. The perforated door of the drum is replaced by a solid door.

A solution is prepared by boiling 9 pounds of the synthetic dyestuff—Pontachrome Brown G (C. I. No. 238) in 50 gallons of water. The dyestuff solution is allowed to cool to a temperature of 100° F. Three pounds of fustic tanning extract are added to the synthetic dyestuff solution. The resulting solution constitutes the dyebath. The dyebath is added, in one addition through the hollow trunnion, to the revolving drum containing the partially-tanned sheepskin skivers. The partially-tanned sheepskin skivers are drummed in the dyebath for 30 minutes at a temperature of 100° F.

A solution is prepared by dissolving 12 pounds of muriatic acid (approximately 32% hydrochloric acid) in 10 gallons of water at 100° F. This solution is slowly added through the hollow trunnion to the revolving drum containing the dyed partially tanned sheepskin skivers. The drumming is continued for 20 minutes. The solid door of the drum is replaced by a perforated door. The drum is revolved until the excess liquor has drained from the drum. The perforated door is replaced by a solid door.

A tanning bath is prepared by boiling together in 8 gallons of water, 36 pounds of commercially prepared basic chromium sulfate (containing 23.2% of chromium calculated as Cr<sub>2</sub>O<sub>3</sub>) and 18 pounds of sodium formate and allowing the resulting solution to stand several hours before adding 40 gallons of water. This tanning bath is added, in one addition through the hollow trunnion, to the revolving drum containing the dyed, partially tanned sheepskin skivers. The drumming is continued for 60 minutes at a temperature of 80° F.

A solution is prepared by dissolving 5 pounds of sodium bicarbonate in 10 gallons of water at a temperature of 80° F. This solution is added, in one addition through the hollow trunnion, to the revolving drum containing the dyed, completely tanned sheepskin skivers. The drumming is continued for 30 minutes at a temperature of 80° F.

The solid door of the drum is replaced by a perforated door. Water at 100° F. is allowed to flow through the revolving drum containing the dyed, tanned sheepskin skivers for 30 minutes. The temperature of the rinsing water is raised to 140° F., and the rinse is continued for 10 minutes.

An emulsion is prepared by stirring into 60 gallons of water at a temperature of 140° F., 30 pounds of a partially sulfonated cod oil (comprising approximately 65% sulfonated cod oil, 15% unsulfonated cod oil and 20% water). This emulsion constitutes the fatliquor. The fatliquor is added, in one addition through the hollow trunnion, to the revolving drum containing the rinsed, dyed, fully-tanned sheepskin skivers. The drumming is continued for 30 minutes at a temperature of 140° F. The fatliquor, fully-tanned, dyed sheepskin skivers are removed from the drum and hoisted-up to drain.

The drained, fatliquored, fully-tanned, dyed sheepskin skivers are "crusted-out" (dried) at a temperature not exceeding 120° F.

The crusted, dyed, tanned sheepskin skivers prepared according to the above process may be used as glove leather. It is characterized by a

soft, level tan color that is unusually fast to washing.

Crusted glove leather prepared from pickled sheepskin skivers by the above method has markedly higher tensile strength, smoother-grain and plumper feel than corresponding leather prepared by prior art methods.

The invention is not limited to the process of preparing leather from pickled sheepskins. It may be applied to other pickled skins. For example, it may be applied to cowhides, horse-hides, deerskins, pigsskins, peccary skins, goatskins, calfskins, cabretta skins and other skins suitable for the manufacture of chrome-tanned leather. Furthermore, the present invention is not limited to the manufacture of chrome-tanned grain garment leather. It may be used for manufacturing other types of chrome-tanned leather. For example, it may be used for manufacturing 10 sueded glove leather, sueded garment leather, sueded shoe leather, grain glove leather, grain shoe leather, and other types of chrome-tanned leather. Further types of leather which may be manufactured by the present invention will be apparent.

As many apparently widely different embodiments of this invention may be made without departing from the spirit and scope thereof, it is to be understood that I do not limit myself to the specific embodiments thereof except as defined in the appended claims.

I claim:

1. The process which comprises subjecting a pickled skin having a pH value of about 2.0 at a temperature of about 80° F. for about ten minutes to the action of a salt solution; tanning it in a chrome bath containing basic chromium sulfate and sodium formate at about 80° F. for about ninety minutes; treating the skin with sodium bicarbonate solution at about 80° F. for about thirty minutes; dyeing the skin with an acid dye; tanning with a vegetable tanning extract; acidifying; completing the tanning with a chrome tan bath containing basic chromium sulfate and sodium formate at about 80° F. for about an hour; neutralizing with sodium bicarbonate; and fatliquoring.

2. The process which comprises subjecting a pickled skin having a pH value of about 2.0 to the action of a salt solution; tanning it incompletely in a chrome tan bath containing sodium formate; neutralizing; dyeing the skin with an acid dye; acidifying; completing the chrome tanning with a tan bath containing sodium formate; neutralizing; and fatliquoring.

3. The process which comprises tanning a pickled skin having a pH value of about 2.0 incompletely in a chrome tan bath containing sodium formate; dyeing the skin with an acid dye; completing the chrome tanning with a tan bath containing sodium formate; and fatliquoring.

4. The process which comprises tanning a pickled skin incompletely in a chrome tanning bath containing a masking agent, dyeing the skin with an acid dye, completing the chrome tanning with a chrome tanning bath containing a masking agent, and fatliquoring.

5. The process of preparing a colored tanned leather which comprises tanning the material incompletely in a chrome tanning bath containing a masking agent, dyeing with an acid dye, and completing the tanning.

6. The process of preparing a colored tanned leather which comprises tanning the material

incompletely in a chrome tanning bath, dyeing with an acid dye, and completing the tanning.

7. The process which comprises subjecting a pickled skin having a pH of about 2.0 to the action of a salt solution, tanning it in a chrome bath containing basic chromium sulfate and sodium formate, treating the skin with sodium bicarbonate solution, dyeing the skin with an acid dye, tanning it with a vegetable tanning extract, acidifying it, completing the tanning with a chrome tan bath containing basic chromium sulfate and sodium formate, neutralizing it, and fatliquoring it.

8. The process which comprises partially tan-

ning a skin with a solution comprising a chromium salt which exhibits tanning properties and an organic acid salt selected from the group consisting of sodium formate, sodium acetate, sodium lactate, sodium oxalate, sodium glycolate and sodium adipate, dyeing the skin with a dye selected from the group consisting of acid and direct dyes, and completing the tanning with a solution comprising a chromium salt which exhibits tanning properties and an organic acid salt from the group consisting of sodium formate, sodium acetate, sodium lactate, sodium oxalate, sodium glycolate and sodium adipate.

DONALD T. KIRBY.

CERTIFICATE OF CORRECTION.

Patent No. 2,303,477.

December 1, 1942.

DONALD TAYLOR KIRBY.

It is hereby certified that error appears in the printed specification of the above numbered patent requiring correction as follows: Page 3, first column, line 34, for "retaining" read --retanning--; page 5, first column, line 67, for "flatliquor" read --flatliquor--; and second column, line 70, for "CR203" read --CR<sub>2</sub>O<sub>3</sub>--; page 8, first column, line 42, for "80% F." read --80° F.--; and that the said Letters Patent should be read with this correction therein that the same may conform to the record of the case in the Patent Office.

Signed and sealed this 2nd day of February, A. D. 1943.

(Seal)

Henry Van Arsdale,  
Acting Commissioner of Patents.